

# United States Patent

Ecer

[15] 3,649,255

[45] Mar. 14, 1972

[54] **CORROSION-RESISTANT NICKEL-MOLYBDENUM ALLOYS**

[72] Inventor: Gunes M. Ecer, Pittsburgh, Pa.  
[73] Assignee: Cyclops Corporation, Universal Cyclops  
Specialty Steel Div., Pittsburgh, Pa.  
[22] Filed: May 25, 1970  
[21] Appl. No.: 40,460

[52] U.S. Cl.....75/170, 75/171  
[51] Int. Cl.....C22c 19/00  
[58] Field of Search .....75/170, 171; 148/32, 32.5

[56] **References Cited**

UNITED STATES PATENTS

1,836,317 12/1931 Franks.....75/171

2,959,480 11/1960 Flint .....75/170

*Primary Examiner*—Richard O. Dean  
*Attorney*—Webb, Burden, Robinson & Webb

[57] **ABSTRACT**

Nickel-molybdenum alloys having increased corrosion resistance and resistance to impact at room temperature and below resulting from a critical control of the amounts of carbon, silicon, vanadium, boron and zirconium without creating vanadium stabilization. The carbon and silicon are maintained in negligible amounts and the vanadium, boron and zirconium are closely controlled.

**2 Claims, No Drawings**

## CORROSION-RESISTANT NICKEL-MOLYBDENUM ALLOYS

### BACKGROUND

Nickel-molybdenum alloys are known to be especially suited for construction of equipment for chemical plants because of their high corrosion resistance to various acids and their good physical properties at room temperature and above. These alloys are known to have excellent resistance to the corrosive attack of hydrochloric acid, phosphoric acid, sulfuric acid and all types of organic acids.

The usual techniques for fabricating chemical plant equipment, such as tanks and pipes involves welding. Welding, which subjects portions of the alloys to high temperatures results in reduced intergranular corrosion resistance near the welded joints. The poor corrosion resistance after welding may be overcome in nickel-molybdenum alloys by a post-weld heat treatment comprising heating the fabricated alloys at a temperature in the range of 900° to 1,175° C. for about 2 to 72 hours. However, this treatment introduces practical problems, which are obvious to metallurgists, for example, scaling and distortion, due to expansion stresses on heating and cooling. This technique for restoring resistance to intergranular corrosion through postweld heat treatment has not enjoyed wide popularity.

Another technique for avoiding intergranular corrosion in nickel-molybdenum alloys after welding has been "vanadium stabilization." This technique is described, for example, in U.S. Pat. No. 2,959,480, issued to G. N. Flint. Basically, vanadium ranging in amounts from 1.1 to 2.3 percent is incorporated in the alloy, which in some manner not entirely understood, prevents the welded nickel-molybdenum alloy from becoming vulnerable to intergranular corrosion. Vanadium stabilized alloys have drawbacks: Because of their compositions, they have not developed their ultimate corrosion resistance and notch toughness, especially at room temperature and below.

In recent years the growth of cryogenic applications, such as the manufacture of liquified gases, has created a demand for chemical plant equipment that has the requisite mechanical strength at cryogenic temperatures defined herein as below 0° C. Most alloys are very brittle at these temperatures and, therefore, unsuitable for these applications.

It has now been discovered that nickel-molybdenum alloys with the improved corrosion resistance and very good low temperature impact strength, as measured by notch ductility tests, can be obtained by close control of the amounts of carbon, silicon, vanadium, boron and zirconium present in nickel-molybdenum alloys but without vanadium stabilization as already described. Alloys according to this invention are advantageous, because they are resistant to intergranular corrosion when welded and do not need a postwelding solution treatment. Further, these alloys have good tensile properties, and high impact strength at room temperatures and cryogenic temperatures and good workability. Alloys according to this invention have corrosion resistance superior to vanadium stabilized alloys before and after welding.

### THE INVENTION

Briefly, according to this invention, there is provided an alloy comprising molybdenum from 20 to 40 percent by weight, iron up to 10 percent, cobalt up to 4 percent, chromium up to 5 percent, manganese up to 2 percent, phosphorous up to 0.03 percent, sulphur up to 0.03 percent, carbon up to 0.1 percent, silicon up to 0.1 percent, vanadium from 0.1 to 1.0 percent, boron from 0.001 to 0.035 percent, zirconium from 0.01 to 1 percent, and the remainder nickel plus incidental impurities.

According to a preferred embodiment of this invention, an alloy is provided comprising 26 to 32 percent by weight molybdenum, up to 7 percent iron, up to 2.5 percent cobalt, up to 1 percent chromium, up to 1 percent manganese, up to 0.025 percent phosphorous, up to 0.03 percent sulphur, up to

0.03 percent carbon, up to 0.03 percent silicon, from 0.2 to 0.8 percent vanadium, from 0.001 to 0.02 percent boron, from 0.01 to 0.1 percent zirconium, and the remainder nickel and incidental impurities.

### EXAMPLE

A 3,000 pound heat of an alloy, according to this invention, hereafter referred to as alloy A, was prepared. To insure a silicon- and carbon-free composition, the heat was melted under vacuum using raw materials relatively free of these elements. While in this example the melt was prepared using vacuum techniques, with other proper melting techniques the improvements mentioned herein would be attainable. The chemical analysis of the ingots cast from the melt was as follows: carbon 0.002 percent, manganese 0.460 percent, silicon less than 0.010 percent, sulphur 0.010 percent, phosphorous 0.002 percent, molybdenum 26.900 percent, iron 5.250 percent, cobalt 1.010 percent, vanadium 0.240 percent, chromium 0.140 percent, boron 0.0025 percent, zirconium 0.029 percent, the balance nickel, except for incidental trace impurities including magnesium, calcium and oxygen.

The ingots cast from the melt had 11-inch × 15-inch cross sections. These ingots were hot forged (1,900° to 2,175° F.) into 3.4-inch × 11-inch slabs. The slabs were hot-rolled to 1/4-inch-thick plates, annealed and pickled. The good hot workability of alloy A, according to this invention, enabled it to be broken down and rolled using well-known techniques.

### COMPARATIVE TESTING

The properties, both physical and chemical, of the alloy A, were ascertained and compared with the properties of two related nickel-molybdenum alloys having the chemical compositions set forth in the following table:

TABLE I

|                 | Comparative<br>Alloy B<br>Nickel-molybdenum<br>alloy - vanadium<br>stabilized | Comparative<br>Alloy C<br>Nickel-molybdenum<br>alloy |
|-----------------|-------------------------------------------------------------------------------|------------------------------------------------------|
| 45 Carbon (C)   | 0.03%                                                                         | 0.05 max.                                            |
| Manganese (Mn)  | 0.48%                                                                         | 1.0 max.                                             |
| Silicon (Si)    | 0.24%                                                                         | 1.0 max.                                             |
| Sulphur (S)     | 0.008%                                                                        | 0.04 max.                                            |
| Phosphorous (P) | 0.017%                                                                        | 0.04 max.                                            |
| Molybdenum (Mo) | 26.92%                                                                        | 28.0                                                 |
| Iron (Fe)       | 5.43 %                                                                        | 5.0                                                  |
| Cobalt (Co)     | 0.38%                                                                         | 2.5 max.                                             |
| Vanadium (V)    | 2.06%                                                                         | 0.2 to 0.6                                           |
| Chromium (Cr)   | 0.19%                                                                         | 1.0 max.                                             |
| Boron (B)       | 0.0112%                                                                       | nil                                                  |
| Zirconium (Zr)  | nil                                                                           | nil                                                  |
| Nickel (Ni)     | balance                                                                       | balance                                              |

Corrosion testing samples of alloy A and comparative alloy B were prepared from solution treated (2,165° F. — 20 minutes — water quench) plates with dimensions of 1/4-inch × 7 1/2-inches × 6 inches. Some samples were tested as is while others were TIG welded using pure tungsten electrodes under an argon atmosphere. One sample plate of each alloy was given a single pass of the welding electrode and another sample of each alloy was given three passes of the electrode. The unwelded and welded plates were then sectioned into 1/4-inch × 1/2-inch × 1/4-inch sections. The sections of the welded plates included the weld bead. Each specimen was surface ground on all faces, including the weld bead, ultrasonically degreased in 70 freon fluorocarbon and cleaned in a 10 percent nitric acid solution.

The dimensions of the corrosion samples were measured to the nearest thousandth of an inch. They were weighed in grams to the fourth decimal place. The samples were tested for corrosion in boiling 20 percent hydrochloric acid, boiling

85 percent phosphoric acid and boiling 20 percent formic acid.

After corrosion testing, from the density of the samples, the

Alloy A and the vanadium stabilized alloy B have comparable tensile properties up to at least 1,200° F. Comparative room temperature tensile data is given in the following table:

TABLE III.—TENSILE DATA (ROOM TEMPERATURE TESTS)

| Grade and condition                                                  | Ultimate tensile strength (p.s.i.) | 0.2% off-set yield strength (p.s.i.) | Elongation in 1" | Reduction of area |
|----------------------------------------------------------------------|------------------------------------|--------------------------------------|------------------|-------------------|
| Alloy A, 0.6 inch plate:<br>2,100° F., 15 min., WQ (transverse)..... | 127,200                            | 54,800                               | 68.6             | 77.0              |
| 2,150° F., 15 min., WQ:<br>Longitudinal.....                         | 125,500                            | 52,900                               | 69.3             | 78.7              |
| Transverse.....                                                      | 124,800                            | 52,400                               | 69.1             | 77.8              |
| 2,200° F., 15 min., WQ (transverse).....                             | 125,000                            | 54,100                               | 72.2             | 77.7              |
| Alloy B:<br>2,165° F., WQ:<br>0.375 inch plate.....                  | 127,200                            | 55,500                               | 66.0             | .....             |
| 0.750 inch plate.....                                                | 123,400                            | 59,800                               | 57.8             | .....             |

\*Values obtained from Union Carbide's preliminary data publication "Hastelloy Alloy B-282" 1967.

specimen dimensions or initial surface area and the weight loss due to corrosion, the corrosion rates were calculated with well-known computations. The results are given in table II.

Impact tests using the Charpy (single beam) impact device were made on alloy A and alloy B at room temperature and at cryogenic temperatures. Standard size V-notch Charpy im-

TABLE II.—CORROSION PROPERTIES

| Acid                                 | Sample                                                           | Corrosion rates |         |
|--------------------------------------|------------------------------------------------------------------|-----------------|---------|
|                                      |                                                                  | I.p.m.          | I.p.y.  |
| 20% hydrochloric acid (boiling)..... | Alloy A, $\frac{1}{4}$ inch plate (2,165° F.-20 min.-WQ).....    | 0.0032          | 0.0380  |
|                                      | Alloy A, .08 inch sheet (2,125° F.-20 min.-WQ).....              | 0.0019          | 0.0229  |
|                                      | Alloy B, $\frac{1}{4}$ inch plate (2,165° F.-20 min.-WQ).....    | 0.0038          | 0.0447  |
|                                      | Alloy A, $\frac{1}{4}$ inch plate, as-welded (one pass).....     | 0.0007          | 0.0082  |
|                                      | Alloy B, $\frac{1}{4}$ inch plate, as-welded (one pass).....     | 0.0010          | 0.0160  |
|                                      | Alloy A, $\frac{1}{4}$ inch plate, as-welded (three passes)..... | 0.0032          | 0.0389  |
|                                      | Alloy B, $\frac{1}{4}$ inch plate, as-welded (three passes)..... | 0.0043          | 0.0518  |
| 85% phosphoric acid (boiling).....   | Alloy A, $\frac{1}{4}$ inch plate (2,165° F.-20 min.-WQ).....    | 0.00030         | 0.0049  |
|                                      | Alloy B, $\frac{1}{4}$ inch plate (2,165° F.-20 min.-WQ).....    | 0.00057         | 0.00746 |
| 20% formic acid (boiling).....       | Alloy A, $\frac{1}{4}$ inch plate (2,165° F.-20 min.-WQ).....    | 0.0009          | 0.0116  |
|                                      | Alloy B, $\frac{1}{4}$ inch plate (2,165° F.-20 min.-WQ).....    | 0.0016          | 0.0176  |

Table II established that alloy A, according to this invention, has better corrosion resistance than the vanadium stabilized alloy B in the solution treated or after welded condition. Alloy A is also superior to alloy C (not vanadium stabilized) in the solution treated condition according to published data for the comparative alloy, which gives the corrosion rate in 85 percent phosphoric acid as 0.028 I.P.Y. (Union Carbide Technical Brochure, "Hastelloy-Corrosion Resistant Alloys"

40 impact specimen were prepared from solution treated 0.6-inch-thick plates of the new alloy A. More notched and unnotched subsized specimens (0.225 inches  $\times$  0.225 inches  $\times$  2.165 inches with V-notch depth 0.050 inches) were prepared from  $\frac{1}{4}$ -inch-thick solution treated alloy A and alloy B. These specimens were tested at room temperature, at -120° F. and -320° F. The results of these tests are given in table IVA and 45 table IVB.

TABLE IVA.—IMPACT TESTING-STANDARD SIZE SAMPLES

| Grade and condition                                      | Test temperature (° F.) | Charpy V-notch impact strength (ft.-lbs.) | Fraction ductile (percent) | Lateral contraction (percent) | Comments       |
|----------------------------------------------------------|-------------------------|-------------------------------------------|----------------------------|-------------------------------|----------------|
| Alloy A, 0.6 inch plate annealed 2,150° F., 15 min., WQ. | Room.....               | >240                                      | 100                        | 26.0                          | Did not break. |
|                                                          | -120.....               | >240                                      | 100                        | 25.3                          | Do.            |
|                                                          | -320.....               | >240                                      | 100                        | 24.6                          | Do.            |
| Alloy B, 0.750 inch plate annealed 2,165° F., WQ.        | Room.....               | * 78                                      | .....                      | .....                         | .....          |
|                                                          | do.....                 | * 58-62                                   | .....                      | .....                         | .....          |

\*Data obtained from Union Carbide's brochures, *supra*.

May, 1967). Furthermore, alloy A possesses the same high corrosion resistance even in as-welded condition, whereas alloy C's susceptibility to intergranular corrosion after welding is well known.

The optimum recommended annealing temperature for alloy B is 2,165° F., whereas for alloy A the optimum temperature has been found to be 2,125° F. Table II directly compares the corrosion resistance of alloy A with alloy B after a 2,165° F. annealing treatment. Data are also set forth in table II showing the corrosion resistance of alloy A after annealing at its optimum annealing temperature. Thus, alloy A is considerably 70 superior to alloy B in corrosion resistance when each alloy is given its optimum annealing treatment.

The lower optimum annealing temperature for alloy A facilitates heat-treating procedures. The lower temperature minimizes warpage and surface oxidization (scaling). Also, the lower temperature is more easily achieved in most industrial shops.

TABLE IVB.—IMPACT TESTING—SUBSIZE SAMPLES

| Grade and condition                               | Specimen       | Test temperature (° F.) | Fracture mode*       |
|---------------------------------------------------|----------------|-------------------------|----------------------|
| Alloy A, 0.250 inch plate (2,165° F.-20 min.-WQ). | Unnotched..... | Room.....               | Did Not Crack.       |
|                                                   | Notched.....   | do.....                 | Do.**                |
|                                                   | do.....        | -120.....               | Do.                  |
|                                                   | do.....        | -120.....               | Do.                  |
|                                                   | Unnotched..... | -320.....               | Do.                  |
| Alloy B, 0.250 inch plate (annealed).             | Notched.....   | Room.....               | Did Not Crack.       |
|                                                   | do.....        | -120.....               | Brittle fracture***. |
|                                                   | do.....        | -120.....               | Do.                  |
|                                                   | Unnotched..... | -320.....               | Did Not Crack.       |
|                                                   | Notched.....   | -320.....               | Brittle fracture***. |

\*Specimens were too thin to break completely.

\*\*Notches opened up slightly in a ductile manner.

\*\*\*Cracked at notches approximately 90% of specimen thickness in a brittle manner.

Table IVA and table IVB establish that alloy A, according to this invention, has unusually superior impact properties, both at room temperature and down to -320°F.

The scientific basis for the improved corrosion resistance and impact strength of nickel-molybdenum alloys, according to this invention, is not entirely understood. However, it is believed that substantial elimination of carbon and silicon and the presence of boron, zirconium, and vanadium in controlled amounts contribute to the homogeneity of the alloy by preventing grain boundary precipitation of detrimental secondary phases and by establishing a more stable chemical and electronic balance which prevents migration of deleterious trace elements to the grain boundaries. The beneficial structural stability is achieved without the aid of vanadium stabilization.

Having thus defined the invention with the detail and particularity required by the Patent Statutes what is desired protected by Letters Patent is set forth in the following claims.

I claim:

1. An alloy having improved corrosion resistance and im- 20

pact strength at room temperature and below consisting essentially of molybdenum from 20 to 40 percent by weight, iron up to 10 percent, cobalt up to 4 percent, chromium up to 5 percent, manganese up to 2 percent, phosphorous up to 0.03 percent, sulphur up to 0.03 percent, carbon up to 0.1 percent, silicon up to 0.1 percent, vanadium from 0.1 to 1 percent, boron from 0.001 to 0.035 percent, zirconium from 0.01 to 1 percent, and the remainder nickel plus incidental impurities.

2. An alloy having improved corrosion resistance properties and improved impact properties at room temperature and below consisting essentially of 26 to 32 percent molybdenum by weight, up to 7 percent iron, up to 2.5 percent cobalt, up to 1 percent chromium, up to 1 percent manganese, up to 0.025 percent phosphorous, up to 0.03 percent sulphur, up to 0.03 percent carbon, up to 0.03 percent silicon, from 0.2 to 0.8 percent vanadium from 0.001 to 0.02 percent boron, and from 0.01 to 0.1 percent zirconium, and the remainder nickel and incidental impurities.

\* \* \* \* \*

25

30

35

40

45

50

55

60

65

70

75